



US006016601A

# United States Patent [19]

Takemoto et al.

[11] Patent Number: 6,016,601

[45] Date of Patent: \*Jan. 25, 2000

[54] **METHOD OF PREPARING THE NOZZLE PLATE**[75] Inventors: **Kiyohiko Takemoto; Miharu Yoshida; Shuichi Yayaguchi; Takeshi Kobayashi; Masanori Kamijo; Akio Yamamori**, all of Nagano, Japan[73] Assignee: **Seiko Epson Corporation**, Tokyo, Japan

[\*] Notice: This patent issued on a continued prosecution application filed under 37 CFR 1.53(d), and is subject to the twenty year patent term provisions of 35 U.S.C. 154(a)(2).

[21] Appl. No.: 08/653,780

[22] Filed: May 28, 1996

**Related U.S. Application Data**

[63] Continuation of application No. 08/127,480, Sep. 28, 1993.

**Foreign Application Priority Data**Mar. 28, 1991 [JP] Japan ..... 3-89522  
Mar. 19, 1992 [JP] Japan ..... 4-93720[51] **Int. Cl.<sup>7</sup>** ..... B41J 2/16  
[52] **U.S. Cl.** ..... 29/890.1; 347/47  
[58] **Field of Search** ..... 29/890.1; 347/47**References Cited****U.S. PATENT DOCUMENTS**4,296,421 10/1981 Hara ..... 347/140 R  
4,343,013 8/1982 Bader ..... 347/47  
4,368,476 1/1983 Uehara ..... 347/45  
4,425,777 1/1984 Jeglinski ..... 29/890.1 X  
4,658,269 4/1987 Rezanka ..... 347/45  
4,728,392 3/1988 Miura ..... 347/47

|           |         |                     |            |
|-----------|---------|---------------------|------------|
| 4,733,447 | 3/1988  | Ageishi .....       | 347/47     |
| 4,849,773 | 7/1989  | Owataru .....       | 347/100    |
| 4,890,126 | 12/1989 | Hotomi .....        | 347/45     |
| 5,016,024 | 5/1991  | Lam et al. .....    | 29/890.1 X |
| 5,426,458 | 6/1995  | Wenzel et al. ..... | 29/890.1 X |

**FOREIGN PATENT DOCUMENTS**

|           |         |                      |          |
|-----------|---------|----------------------|----------|
| 0359365   | 3/1990  | European Pat. Off. . |          |
| 55-65564  | 5/1980  | Japan .              |          |
| 55-148170 | 11/1980 | Japan .              |          |
| 57-22068  | 2/1982  | Japan .              |          |
| 57-107848 | 7/1982  | Japan .              |          |
| 58-124661 | 7/1983  | Japan .              |          |
| 59-176054 | 10/1984 | Japan .              |          |
| 60-183161 | 9/1985  | Japan .              |          |
| 61-248753 | 11/1986 | Japan .              |          |
| 61-291148 | 12/1986 | Japan .              |          |
| 2-55140   | 2/1990  | Japan .              |          |
| 4368854   | 12/1992 | Japan .....          | 29/890.1 |

*Primary Examiner*—Lee Young*Assistant Examiner*—Rick Kiltae Chang*Attorney, Agent, or Firm*—Sughrue, Mion, Zinn, Macpeak & Seas, PLLC

[57]

**ABSTRACT**

The entire part of a rear surface 2 of a nozzle plate 1 excluding peripheral portions 6 of nozzle holes 4 is coated with a resist tape, and this nozzle plate 1 is immersed in an electrolytic solution in which ions of a metal and particles of a water-repellent resin are dispersed to provide a plating thereon, and the plated nozzle plate 1 in the electrolytic solution is then heated to a temperature that is higher than a melting point of the water-repellent resin, whereby an entire portion extending from a front surface 3 of the nozzle plate 1 and the nozzle holes 4 contiguous to the front surface to the rear surface 2 is provided with a eutectoid plating layer 8 to suppress deviation of the passage of ink droplets due to wetting by an ink or the like.

**14 Claims, 2 Drawing Sheets**

FIG. 1



FIG. 3(a)



FIG. 3(b)



FIG. 3(c)



FIG. 2(a)



FIG. 2(b)



FIG. 2(c)



FIG. 2(d)



FIG. 2(e)



## METHOD OF PREPARING THE NOZZLE PLATE

This is a Continuation of application Ser. No. 08/127, 480, filed Sep. 28, 1993, now pending.

### BACKGROUND OF THE INVENTION

#### 1. Field of the Invention

The invention relates to a nozzle plate adapted for an ink jet recording apparatus and a method of preparing such nozzle plate. More particularly, it is directed to a nozzle plate on which a water-repellent coating is provided on both the front surface of the nozzle plate and on the inner surface of the nozzles and to a method of preparing such nozzle plate.

#### 2. Prior Art

An ink jet printer has a problem that when a portion around a nozzle is wetted by an ink, the direction of splashing ink droplets deviates. To overcome this problem, Japanese Patent Unexamined Publication No. 65564/1980 or 55140/1990 has proposed an art that contributes to suppressing generation of such wetting by the ink while providing a water-repellent coating on the surface of the nozzle plate.

However, to form such a coating, the rear surface of the nozzle plate must be masked to facilitate adhesion of an adhesive. With nozzle holes having been arranged on a member to be coated, it is difficult to cover a portion around the holes completely. Under such circumstances, part of the water-repellent coating provided on the front surface is extended into the inner surfaces of the nozzle holes unevenly, making the ink meniscuses to be formed inside the respective nozzle holes to be different from one nozzle hole to another and disadvantageously causing variations in ink jetting timing.

Further, a technique in which a coating material is embedded in each nozzle hole completely so that a water-repellent coating is provided only on the front surface of the nozzle plate causes the coating to form an edge-like protrusion around the rim portion of each nozzle hole. Thus, when such rim portion is wiped, the edge-like protrusion is chipped off, making the wettability locally different with resultant inconsistent ink splashing directions.

Still further, the provision of the water-repellent film only on the front surface of the nozzle plate causes inconsistent affinity at the exit of each nozzle hole, making the meniscus position unstable.

### SUMMARY OF THE INVENTION

An object of the invention is to provide a novel nozzle plate that does not cause variations in both the direction of splashing ink droplets and the timing of jetting the ink droplets.

To achieve the above object, the invention is applied to a nozzle plate in which not only the front surface of the nozzle plate but also the inner surface of each nozzle hole are provided with a water-repellent coating uniformly.

Another object of the invention is to allow the meniscus of an ink to be formed more stably inside each nozzle hole.

To achieve this object, the invention is applied to a nozzle plate in which the water-repellent coating extending from the front surface of the nozzle plate to the inner surface of each nozzle plate is further extended to a portion around the ingress of each nozzle hole.

Still another object of the invention is to propose a novel method of forming a coating on a nozzle plate in which a

water-repellent coating is formed uniformly from the portion around the ingress of each nozzle hole not only to the inner surface of the nozzle hole but also to the front surface of the nozzle plate.

To achieve this object, the invention is applied to a method comprising the steps of: providing a coating on the rear surface of a nozzle plate with a coating material excluding each nozzle hole and a portion around such nozzle hole to thereby form a uniform water-repellent coating on the front surface of the nozzle plate, the inner surface of each nozzle hole contiguous to the front surface, and the portion around the nozzle hole contiguous to the rear surface of the nozzle plate.

### BRIEF DESCRIPTION OF THE DRAWINGS

FIG. 1 is an enlarged sectional diagram showing a main portion of a nozzle plate, which is an embodiment of the invention;

FIG. 2(a) to (e) are diagrams showing processes for providing a water-repellent coating onto surfaces of the nozzle plate; and

FIG. 3(a) to (c) are diagrams showing a masking process.

### DETAILED DESCRIPTION OF THE PREFERRED EMBODIMENTS

FIG. 1 shows a nozzle plate, which is an embodiment of the invention, and FIGS. 2(a) to (e) show its preparing processes.

The processes for preparing the nozzle plate will be described first with reference to FIGS. 2(a) to (e).

In FIGS. 2(a) to (e), a nozzle plate 1 is made of such a material as metal, ceramic, silicon, glass, or plastic, and preferably of a single metal such as titanium, chromium, iron, cobalt, nickel, copper, zinc, tin, gold, or of an alloy such as a nickel-phosphor alloy, a tin-copper-phosphor alloy (phosphor bronze), a copper-zinc alloy, or a stainless steel; of polycarbonate, polysulfone, an ABS resin (acrylonitrile butadiene-styrene copolymer), polyethylene terephthalate, polyacetal; and various photosensitive resins. This nozzle plate has a plurality of nozzle holes 4, each consisting of an inverted funnel-like portion on a rear surface 2 and a thinly opened orifice portion on a front surface 3.

In this nozzle plate 1 a resist tape 8 is stuck onto the rear surface 2 as appropriate excluding the nozzle holes 4 and their peripheral portions 6 (FIG. 2(b)).

That is, on the rear surface 2 of the nozzle plate 1 is bonded the resist tape 8, the resist tape 8 having a multiplicity of such large-diameter holes 7 as to allow the funnel-like portions and its peripheral portions 6 to be exposed toward the flat rear surface 2. Each hole 7 may be formed by punching after the resist tape 8 has been bonded onto the nozzle plate 1.

The nozzle plate 1 with the resist tape 8 bonded thereon is cleaned with an acid, and then dipped into an electrolytic solution in which nickel ions and particles of a water-repellent high molecular resin such as polytetrafluoroethylene are dispersed by electric charges to be eutectoid plated on the front surface while stirring the electrolytic solution (FIG. 2(c)).

A fluorine-containing high molecule to be used for the eutectoid plating includes: polytetrafluoroethylene, polyperfluoroalkoxybutadiene, polyfluorovinylidene, polyfluorovinyl, polydiperfluoroalkyl fumarate, and resins shown by the following chemical formulas 1, 2, 3, 4, and 5, used singly or in mixture.



(1)



(2)

where at least two of X1 to X4 are fluorine or perfluoroalkyl group, and R1 to R4 are hydrocarbon substituent (including hydrogen and halogen).



(3)

where R is  $\text{COOC}_m\text{F}_{2m+1}$  ( $m=1-20$ )



(4)

where R is alkyl group.



(5)

where R is alkyl group.

There is no particular limit on the matrix for a coating layer, allowing a metal to be selected from the group consisting of nickel, copper, silver, zinc, tin, and the like. Preferably, however, nickel, a nickel-cobalt alloy, a nickel-phosphor alloy, a nickel-boron alloy, and the like, having good surface hardness and high wear resistance, should be selected.

Accordingly, the particles of polytetrafluoroethylene form a uniform plating on the front surface 3 of the nozzle plate 1, the inner surface 5 of each nozzle hole 4, and the rear surface 2 portion exposed from the hole 7 of the resist tape 8 by means of the nickel ions. Then, while suppressing warpage of the nozzle plate 1 by applying a load to the nozzle plate 1, the nozzle plate 1 in the electrolytic solution is heated to a temperature over the melting point of polytetrafluoroethylene, i.e., 350°C.

As a result, the particles of polytetrafluoroethylene are fused on the front surface 3 of the nozzle plate 1, the inner surface 5 of each nozzle hole 4, and the peripheral portion 6 of the nozzle hole 4, forming there an ink-repellent plating layer 10 that is smooth and hard.

The fluorine-containing high molecule eutectoid plating layer 10, if too thin, exhibits inadequate ink repellency on the surface having an ink jetting outlets, while if too thick, affects accuracy in the diameter of each ink jetting outlet. 5 Therefore, the thickness of the plating 10 on the surface is designed to be controlled in the order of 1 to 10  $\mu\text{m}$ .

Further, it is preferable that the eutectoid amount of fluorine-containing high molecule in the plating layer 10 be up to 60 vol.%, more particularly, from 10 to 50 vol.%. 10

An eutectoid plating method may include electroless plating and electroplating. From the consideration that an ink including an ink jet recording ink is used and that ions such as  $\text{Li}^+$ ,  $\text{Na}^+$ ,  $\text{K}^+$ ,  $\text{Ca}^{2+}$ ,  $\text{Cl}^-$ ,  $\text{SO}_4^{2-}$ ,  $\text{SO}_3^{2-}$ ,  $\text{NO}_3^-$ ,  $\text{NO}_2^-$  are mixed therein as impurities, it is desirable to employ the electroplating method that is less affected by 15 ionic products and provides highly durable plating.

Further, to prevent warpage of the nozzle plate 1 caused when the fluorine-containing high molecule eutectoid plated nozzle plate 1 is heated to a temperature over the melting point of the fluorine-containing high molecule, it is proposed 20 that a pressure of 100  $\text{gf}/\text{cm}^2$  or more, preferably, a pressure of 500  $\text{gf}/\text{cm}^2$ , be applied onto the nozzle plate 1.

The ink-repellent plating layer 10 formed on the front surface 3 of the nozzle plate 1 and the inner surface 5 of each nozzle hole 4 in this way further reaches the rear surface 2 of the nozzle plate 1, where it is spread over the peripheral portion 6 of each nozzle hole 4. 25

As a result, the entire part of a portion extending from the periphery to the inner portion of each nozzle hole 4 exhibits a uniform surface condition, so that the meniscus M oscillates largely by, e.g., a variation in the pressure within an ink 30 chamber, and even if this causes the meniscus M to retreat toward the ink chamber in the vicinity of the funnel-like portion as shown in FIG. 1, the stable spherical surface of the meniscus M is maintained, allowing a high-frequency recording and writing to be made without causing deviation 35 in the passage of ink droplets nor omission of dots.

Therefore, as the resist tape 8 is removed from the rear surface 2 of the nozzle plate 1 thereafter and the nozzle plate 1 is adhesively fixed on a substrate 12 while applying an adhesive 11 on the portion from which the tape was 40 removed, so that an ink jet recording head is implemented.

FIGS. 3(a) to (c) show another means for coating the rear surface 2 of the nozzle plate 1.

As in the ordinary masking method, this coating means involves the steps of applying a liquid resist material 18 over 45 the entire part of the rear surface 2 of the nozzle plate 1 (FIG. 3(a)), then exposing the peripheral portion 6 (FIG. 3(b)), and removing by fusion the exposed portion. As a result, as shown in FIG. 3(c), only the portion to which the adhesive 19 was applied can be coated.

While this coating means is employed to provide the above-mentioned eutectoid plating layer 10 on the nozzle plate 1, ink-repellent coating forming means other than this can, of course, be used.

Specifically, ink-repellent coating forming means other 55 than the above includes a method of applying a fluororesin by dipping. While this ink-repellent coating has a shortcoming that it is weak to externally applied mechanical action such as wiping compared with the eutectoid plating, this coating with its low melting point allows the nozzle plate 1 to be made from a material that is comparatively less heat-resistant such as a synthetic resin.

What is claimed is:

1. A method of manufacturing an inkjet recording head, comprising:  
65 immersing a nozzle plate in an electrolyte to form an ink-repellent layer formed of an eutectoid plating layer on at least a surface of said nozzle plate;

**5**

then heating nozzle plate with ink-repellent layer to form an ink-repellant coating;  
 applying pressure to said nozzle plate to prevent warping of said nozzle plate; and  
 then fixing said nozzle plate to a substrate. 5  
**2.** The method according to claim 1, wherein said heating step and said step of applying pressure are performed simultaneously.  
**3.** The method according to claim 1, wherein said forming step comprises the step of forming a fluorine-containing high molecular coating. 10

**4.** The method according to claim 1, wherein said forming step comprises the step of forming a fluorine-containing high molecule eutectoid plating. 15

**5.** The method according to claim 1, wherein step of applying pressure comprises the step of applying a pressure of at least 100 gf/cm<sup>2</sup>. 15

**6.** The method according to claim 1, wherein said fixing step comprises the step of adhering said nozzle plate to said substrate. 20

**7.** A method as claimed in claim 1, wherein said electrolyte is obtained by diffusing grains of high-polymer resin and metal ions. 25

**8.** A method as claimed in claim 1, wherein said electrolyte is obtained by diffusing grains of high-polymer resin and nickel ions. 25

**9.** A method of manufacturing a nozzle plate for an ink jet recording head, comprising: 30

forming an ink-repellant coating film on a front surface of said nozzle plate inner surfaces of nozzle holes formed in said nozzle plate, and on a portion of said nozzle holes which is contiguous with a rear surface of said nozzle plate;

then heating said ink-repellant coating film formed on said nozzle plate;

**6**

applying pressure to said nozzle plate to prevent warping of said nozzle plate; and  
 then fixing said nozzle plate to a substrate; 5  
 wherein said forming step comprises:

applying resist tape onto predetermined areas of said rear surface of said nozzle plate so as to expose peripheral portions on said rear surface leading to said nozzle holes and inner surfaces of said nozzle holes; and  
 dipping said nozzle plate into an electrolyte solution to produce an eutectoid plated surface on said front surface of said nozzle plate, said inner surface of said nozzle holes, and on said rear surface of said nozzle plate at areas other than said predetermined covered areas by said resist tape. 15

**10.** The method according to claim 9, wherein said step of applying pressure to said nozzle plate and said heating step are performed simultaneously. 15

**11.** The method according to claim 9, wherein said fixing step comprises the steps of: 20

removing said resist tape; and  
 adhering said nozzle plate onto said substrate. 25

**12.** The method according to claim 9, wherein said forming step comprises the step of forming said ink-repellent coating film comprising a fluorine-containing high molecular coating. 25

**13.** The method according to claim 9, wherein said forming step comprises the step of forming said ink-repellent coating film comprising a fluorine-containing high molecule eutectoid plating. 30

**14.** The method according to claim 9, wherein said step of applying pressure comprises the step of applying a pressure of at least 100 gf/cm<sup>2</sup>. 35

\* \* \* \* \*

UNITED STATES PATENT AND TRADEMARK OFFICE  
**CERTIFICATE OF CORRECTION**

PATENT NO. : 6,016,601  
DATED : January 25, 2000  
INVENTOR(S) : Kiyohiko Takemoto et al.

Page 1 of 1

It is certified that error appears in the above-identified patent and that said Letters Patent is hereby corrected as shown below:

Title page.

Item [75], Inventors: please change the 3<sup>rd</sup> inventor from “**Shuichi Yayaguchi**” to  
-- **Shuichi Yamaguchi** --

Signed and Sealed this

Eleventh Day of February, 2003



JAMES E. ROGAN  
*Director of the United States Patent and Trademark Office*